

# UNITED STATES PATENT OFFICE.

JOHN B. HUFFARD, OF GLEN FERRIS, WEST VIRGINIA, ASSIGNOR TO ELECTRO METALURGICAL COMPANY, OF NEW YORK, N. Y., A CORPORATION OF WEST VIRGINIA.

## PROCESS OF PRODUCING LOW-CARBON METALS AND ALLOYS.

992,422.

Specification of Letters Patent. Patented May 16, 1911.

No Drawing.

Application filed November 14, 1910. Serial No. 592,361.

To all whom it may concern:

Be it known that I, JOHN B. HUFFARD, a citizen of the United States, residing at Glen Ferris, in the county of Fayette and State of West Virginia, have invented certain new and useful Improvements in Processes of Producing Low-Carbon Metals and Alloys, of which the following is a specification.

- 10 This process is designed to effect the reduction of refractory metallic oxids, for example those of tungsten, vanadium, molybdenum and uranium, and the production of substantially carbonless metals and alloys.
- 15 The novel feature of the process is the use of a reducing agent containing titanium in an oxidizable form, either metallic titanium, an oxidizable titanium compound such as the nitrid, oxid or carbid, or a mixture or compound of two or more of these reagents.

According to the preferred process, the titanium reducing agent is first made, as by electrically smelting a mixture of rutile or other titanium ore and carbon. The product may consist of metallic titanium containing relatively small amounts of titanium nitrid, carbid and monoxid. The reagent is then caused to react on the oxid of the desired metal. For this purpose a mixture of the reducing agent and the reducible oxid, both in a divided condition, may be brought to the requisite temperature in an electric furnace. Or the metallic oxid may be gradually fed into a bath of the molten reducing agent.

The principal reactions, taking tungstic oxid as an example, are indicated by the following equations:

- 40 (1)  $2WO_3 + 3Ti = 2W + 3TiO_2$   
(2)  $2WO_3 + 3TiN = 2W + 3TiO_2 + 3N$   
(3)  $WO_3 + 3TiO = W + 3TiO_2$   
(4)  $WO_3 + TiC = W + TiO_2 + CO$

- 45 For the production of low-carbon metals, it is preferable to use a reagent containing a minimum amount of titanium carbid, as the oxidation of the combined carbon is not complete. In order to fully oxidize and 50 utilize all of the titanium, it is necessary to react on an excess of the reducible oxid.

The resulting slags then contain both the oxidized titanium and the unreduced oxid of the charge. Titanium oxid not being acted upon by acids, the unreduced oxid 55 may be dissolved out of the slags and recovered by evaporation for subsequent treatment. Tungstic oxid may be readily dissolved out by hydrochloric acid. By this method, a very high recovery of tungsten 60 and other difficultly-reducible expensive metals may be obtained, while the reducing agent is fully utilized.

If a low-carbon product is not required, the initial production of the titanium-reducing agent and its reaction on the refractory oxid may be effected as successive phases of a single operation, by electrically smelting a mixture of the oxids of titanium and the desired metal with carbon.

For the production of alloys, a titanium-reducing agent containing the desired alloying metal may be used, the titanium being oxidized and the residual metal alloying with the reduced metal.

I claim:

1. The process of reducing refractory metallic oxids, which consists in reacting on the oxid, at the requisite temperature, with a titanium reducing agent.

2. The process of reducing refractory metallic oxids and producing low-carbon metals and alloys, which consists in reacting on the oxid, at the requisite temperature, with a titanium reducing agent low in 85 carbon.

3. The process of treating refractory metallic oxids, which consists in reacting on an excess of the oxid, at the requisite temperature, with a titanium reducing agent, 90 and recovering the unreduced oxid from the slag.

4. The process of reducing refractory metallic oxids and producing alloys, which consists in reacting on the oxid, at the requisite temperature, with a titanium reducing agent containing an alloying metal, thereby oxidizing the titanium and causing the residual metal to combine with the reduced metal.

5. The process of reducing refractory metallic oxids and producing alloys, which con-

sists in reacting on an excess of the oxid, at the requisite temperature, with a titanium reducing agent containing an alloying metal, thereby oxidizing the titanium and 5 causing the residual metal to combine with the reduced metal, and recovering the un-reduced oxid from the slag.

In testimony whereof, I affix my signature in presence of two witnesses.

JOHN B. HUFFARD.

Witnesses:

H. E. KIR,  
ALFRED R. KOCH.